

# UNITED STATES PATENT OFFICE

GIDEON E. MOORE, OF NEW YORK, N. Y.

## PROCESS OF TREATING ORES OF ZINC, MANGANESE, OR IRON.

SPECIFICATION forming part of Letters Patent No. 505,408, dated September 19, 1893.

Application filed March 6, 1893. Serial No. 464,882. (No specimens.)

To all whom it may concern:

Be it known that I, GIDEON E. MOORE, a citizen of the United States, residing in the city of New York, county and State of New York, have invented certain new and useful Improvements in Processes of Treating Ores of Zinc, Manganese, or Iron, of which the following is a specification.

The ores to which my invention especially applies consist of mixtures of minerals containing zinc, manganese and iron or either of these substances, as, for example, willemite, zincite, franklinite, &c., with a gangue consisting essentially or largely of carbonate of lime with smaller proportions of carbonate of manganese or of magnesia, or both, which gangue in the following description will be termed "limestone." In the case of such ores, and notably those occurring in the county of Sussex, New Jersey, these minerals occur in distinct crystals or crystalline particles, often of considerable size, embedded in the gangue and frequently either detached, or so loosely adherent that when the gangue is removed the crystals or granules of the different minerals may, to a considerable extent, be separated from each other by hand sorting, sifting, washing or other simple mechanical means. In the methods of treatment heretofore applied to these ores, the ores have been crushed together with the gangue, and either subjected directly to metallurgical treatment for the recovery of the zinc that they contain, the slags or cinders from the last named treatment being subsequently utilized for the recovery of the iron and manganese, or the crushed ore has been subjected to jigging or other mechanical process of concentration to remove more or less of the gangue previous to the metallurgical treatment. This preliminary crushing, with or without concentration of the ore, is usually done at the reduction works at some distance from the mines and is not only expensive but involves the transportation of the gangue and other worthless portions of the ore, as well as the valuable constituents. Moreover by the process of crushing the valuable constituents of the ore are crushed as well as the gangue, the crushing can rarely be economically carried so far as to insure a perfect separation of the gangue

from the particles of valuable material and the latter are reduced in size by the crushing, which is a condition less favorable for certain of the simpler processes of concentration and metallurgical treatment. For all of these reasons the processes in question have heretofore been profitably employed only with ores of a certain degree of richness in zinc.

The object of my invention is to remove the limestone gangue from these ores, leaving the valuable constituents as nearly as possible in their original condition as to size and shape of particles, so as to facilitate the separation of the individual metalliferous minerals preliminary to their separate metallurgical treatment, the separation of these metalliferous minerals, and their metallurgical treatment for the recovery of the metals that they contain.

In carrying out my invention I proceed as follows, to wit: I take the lump ore as it comes from the mine and, if necessary, break it into pieces of suitable size. In most cases pieces of about eight inches cube, more or less, may be used, although the size is only material in regard to the form, size and mode of operation of the furnace used. I then calcine the ore in a furnace or kiln of any suitable known construction or material, or in heaps, wherein it may be subjected to the action of heat, for the purpose of depriving the limestone of as much of its carbonic acid as may be necessary to give it the property of slaking, or disintegrating, or falling to powder, or to particles of greater or less degree of fineness, when subjected to the action of hot or cold water, or steam, or to prolonged exposure to the atmosphere. For this purpose any known mode of calcination either in furnaces, kilns or heaps, with or without the use of steam, may be employed. It is essential that the ore should not be subjected to a too high heat as that would cause the lime formed during the calcination to act upon the willemite, which is a silicate of zinc, and decompose it nor must the ore be heated in contact with reducing materials or in an atmosphere of reducing gases as that would especially if high temperatures be used lead to a loss of zinc by reduction and volatilization. I have found in practice a dull red

heat and a non-reducing or at most slightly reducing atmosphere to be favorable conditions for this process, and consider a kiln, such as what is known as a perpetual flame 5 kiln, with separate firing and continuous working, a suitable furnace to be used therewith. When properly calcined, I remove the ore and either slake the limestone, or product of calcining the same, by addition of a suitable quantity of hot or cold water or steam, which slaking is most active when performed before the ore has entirely cooled, or I allow the calcined ore to disintegrate by the process 10 known as air-slaking. When properly slaked the mass will be found to consist of slaked or disintegrated gangue with intermixed particles of the willemite, franklinite and zincite the said minerals being almost or entirely unchanged in size of particles and other essential respects from the state in which they 15 were contained in the original ore. After the removal of the gangue the valuable minerals may either be sent directly to the furnaces for reduction or they may, either with or without previous crushing, be subjected to any known 20 process of mechanical separation. When the proportion of gangue is very considerable it is usually convenient to remove more or less of it from the calcined and slaked material by sifting, washing, or other mechanical means 25 before proceeding to separate the individual metalliferous minerals from each other, which may be done by sifting, screening, jiggling or washing, or other known means of separation 30 based on difference in size of particles or specific gravity of the materials to be separated or, if any portion thereof is possessed of magnetic properties, by the use of any known process of magnetic separation 35 employed in the separation of magnetic from non-magnetic materials. When the proportion of gangue is relatively small, especially as compared with the proportion of magnetic substance contained in the calcined and dis- 40 integrated material, it is sometimes expedient to reverse the order of procedure so as to first separate the magnetic portion by magnetic separation and then to separate the non-magnetic portion of the valuable minerals 45 from the calcined and disintegrated gangue. The foregoing process furnishes as a by-product dry or moist slaked lime which may be used for whatever technical application it may be adapted for. 50 When the process of magnetic separation is used the magnetic portion will be found to consist chiefly of compounds of manganese and iron, with more or less zinc. It may be either used directly in the blast furnace in 55 the manufacture of spiegeleisen or, if it be found to be rich in zinc, it may be previously passed through the Wetherill or other furnace to remove more or less of the zinc, and the slags therefrom used in the blast furnace. 60 The zinc compounds will be found chiefly in the non-magnetic portion which may be sub-

jected to any of the known and suitable processes of metallurgical treatment for the extraction of the zinc contained therein.

Having thus described my invention, what I claim as new, and desire to secure by Letters Patent, is—

1. The herein described process of treating ores of zinc, manganese and iron containing willemite and franklinite and contained in a limestone gangue which consists in calcining the ore and the gangue in a practically non-reducing atmosphere, causing the calcined gangue to slake or disintegrate by hydration, separating the willemite and franklinite 75 from the disintegrated gangue and subjecting them to furnace treatment for the recovery of the metals they contain substantially as described.

2. The herein described process of treating ores of zinc, manganese and iron containing willemite and franklinite and contained in a limestone gangue which consists in calcining them in a practically non-reducing atmosphere to render the lime more or less caustic, 80 causing the calcined gangue to slake or disintegrate by hydration, removing the disintegrated gangue, separating the minerals consisting chiefly of compounds of zinc from those consisting chiefly of compounds of manganese 85 and iron and subjecting the several products to separate metallurgical treatment for the recovery of the metals they contain substantially as described.

3. The herein described process of treating ores of zinc, manganese and iron containing willemite and franklinite and contained in a limestone gangue, which consists in calcining them in a practically non-reducing atmosphere to render the gangue more or less caustic, 90 causing the gangue to slake or disintegrate by hydration and separating the magnetic and non-magnetic ores from each other and from the disintegrated gangue substantially as described. 100

4. The herein described process of treating ores of zinc, manganese and iron containing willemite and franklinite and contained in a limestone gangue, which consists in calcining them in a practically non-reducing atmosphere, causing the calcined gangue to slake or disintegrate by hydration, separating the magnetic and non-magnetic ores from each other and from the disintegrated gangue, and subjecting the magnetic and non-magnetic 115 ores to separate metallurgical treatment for the recovery of the metals they contain substantially as described.

5. The herein described process of treating ores of zinc, manganese and iron containing willemite and franklinite and contained in a limestone gangue which consists in calcining them in a practically non-reducing atmosphere to render the gangue more or less caustic, 120 causing the calcined gangue to slake or disintegrate by hydration, removing the disintegrated gangue, separating the magnetic 125

130

from the non-magnetic ores by the use of a magnetic separator and subjecting the magnetic and non-magnetic ores to separate metallurgical treatment for the recovery of the metals they contain substantially as described.

6. The herein described process of treating ores of zinc, manganese and iron containing willemite and franklinite and contained in a limestone gangue which consists in calcining them in a practically non-reducing atmosphere, causing the calcined gangue to slake or disintegrate by hydration, separating the ore consisting chiefly of compounds of zinc and the ore consisting chiefly of compounds of manganese and iron from each other and from

the disintegrated gangue, smelting the ore consisting chiefly of compounds of manganese and iron in the blast furnace for spiegeleisen and subjecting the ore consisting chiefly of compounds of zinc to metallurgical treatment <sup>20</sup> for the extraction of the zinc substantially as described.

In testimony whereof I have hereunto set my hand and seal in the presence of two subscribing witnesses.

GIDEON E. MOORE. [L. S.]

Witnesses:

T. BROWN, Jr.,  
R. W. MILNE.